

# United States Patent Office

3,103,494

Patented Sept. 10, 1963

1

3,103,494

## LUBRICANT ADDITIVES

Gunter Spengler and Hannsheim Hohn, Munich, Germany, assignors to The Alpha Molykote Corporation, Stamford, Conn.

No Drawing. Filed June 5, 1957, Ser. No. 663,607

Claims priority, application Germany June 28, 1956

16 Claims. (Cl. 252—49.7)

This invention relates to lubricant additives and their preparation.

The excellent lubricating properties of molybdenum compounds have been known for some time. Difficulties have, however, been encountered in attempts to use them as additives in liquid lubricants. These difficulties are due primarily to the general insolubility and high specific gravity of molybdenum compounds. As a result, attempts to use them as additives to liquid lubricants have been more or less limited to formulations for suspending them in oils. Unfortunately, however, such suspensions generally have poor stability because of the high specific gravity of the suspended material.

We have found that phosphomolybdc acid, a compound that is well known as containing molybdenum in sexivalent form, and salts thereof with an organic nitrogen base, can be reduced by reaction with an organic compound to a form in which at least a part of the molybdenum is tetravalent, and that the resulting products possess a very appreciable solubility in an excess of the reducing agent as well as in other chemically related organic compounds. It is surprising that the reduction can be carried out with any organic compound having an active hydrogen in the molecule.

The organic compounds that are suitable for the reduction of phosphomolybdc acid and salts thereof include higher alcohols, esters, glycols and polyalkylene glycols as well as organic nitrogen bases, which can have multiple functions as reducing agents, neutralizing agents, stabilizing agents and further as diluents.

It is advantageous to use, as reducing agents, organic compounds which, by reason of their molecular structure, are soluble in mineral oils or other liquid lubricants or which have lubricating properties of their own. Inasmuch as phosphomolybdc acid as well as its complex reduction products after treatment with most organic reducing compounds are acidic and therefore corrosive, it is desirable to use the salts of phosphomolybdc acid with organic nitrogen bases rather than phosphomolybdc acid per se as a starting material, or to neutralize the acidic products obtained by reduction of phosphomolybdc acid with other organic reducing compounds such as alcohols. Organic nitrogen bases can therefore advantageously be employed in several ways, e.g., to neutralize phosphomolybdc acid and form a salt thereof to be used as a starting material, whereupon a different organic compound such as an alcohol is used as a reducing agent; as a reducing agent for the phosphomolybdc acid, in which instance the organic nitrogen base is preferably used in excess and accomplishes neutralization and reduction; and for neutralizing and heat stabilizing the acidic reaction product of phosphomolybdc acid with a non-basic organic reducing compound, such as an alcohol. It is to be understood of course that the organic nitrogen bases can be used for more than one of these functions.

It is surprising that all known organic nitrogen bases that are soluble in or at least compatible with liquid lubricants are suitable for use in neutralizing and reducing phosphomolybdc acid, and for neutralizing and enhancing the thermal stability of an acidic reaction product of phosphomolybdc acid with a non-basic reducing agent. The extent to which the final reaction products of phosphomolybdc acid with organic nitrogen bases can be

2

used as additives for lubricants depends upon the particular use to which the lubricant is to be put and on the particular conditions thereof such as the nature of the bearing surfaces, temperature and pressure. The same is true also for molybdenum complexes containing non-basic organic reducing compounds which may themselves be lubricants. The organic compounds, including organic nitrogen bases, must of course be at least compatible with the liquid lubricants to which the ultimate product is to be added.

The organic nitrogen bases that are suitable for neutralizing the acidity of phosphomolybdc acid and of the products obtained by reducing the acid with non-basic organic reducing compounds in order that the final additive will not be corrosive to bearing surfaces include such high molecular weight amines as oleylamine; dioleylamine; oleyloxyethylglyoxalidine; dehydroabietylamine; N - aminopropylmorpholine; di - 2 - ethylhexylamine; "Armeen" 2T, believed to be a mixture of secondary amines  $R_2NH$  in which the R's are 30% hexadecyl, 25% octadecyl, and 45% octadecenyl; "Duomeen" C, believed to be a mixture of N-alkylpropylene diamines of the formula  $RNH_2$  in which R is a mixture of saturated alkyl radicals containing eight, ten, twelve, sixteen and eighteen carbon atoms and unsaturated eighteen carbon atom alkyl radicals, the  $C_{12}$  alkyl radicals being predominant; and "Armeen" SD, believed to be a mixture of primary hexadecyl, octadecyl, octadecenyl, octadecadienyl amines. These basic nitrogen compounds may also, as indicated earlier, be used as reducing agents for reducing the valence of at least some of the molybdenum from six to four and converting the complex acid or reaction product into a lubricant-soluble state.

Non-basic organic compounds that are suitable for reducing the valence of the molybdenum from six to four and rendering it lubricant-soluble and which are themselves either soluble in lubricants or are lubricants per se include such higher alcohols, esters, glycols and polyalkylene glycols as ethyl hexanediol, a term intended to include the various isomers thereof including 2-ethyl-1,6-hexanediol; Abitol, a mixture of 15% dehydroabietyl alcohol, 40% dihydroabietyl alcohol and 45% tetrahydroabietyl alcohol; Eutanol, a highly refined liquid mixture of predominantly animal origin containing fourteen to eighteen carbon atoms; normal octadecanol; the diethyl esters of adipic acid; benzylbutyl phthalate; "Ucon" 50-HB660, a water-soluble polyalkylene glycol; "Ucon" DLB-67E, a water-insoluble polyalkylene glycol; "Ucon" 75-H1400, a polyalkylene glycol reported to have a specific gravity of 20/20° C. of 1.093; polyethylene glycol; dibutoxytetraglycol,  $C_4H_9O(C_2H_4O)_4C_4H_9$ ; "Flexol" 4GO,  $C_{11}H_{15}OOCCH_2(CH_2OCH_2)_xCH_2COOC_{17}H_{35}$  having a viscosity of 25.1 cp. at 20° C.; and "Flexol" CC-55,  $C_6H_{10}[COOCH_2CH(C_2H_5)C_4H_9]_2$ .

To convert the phosphomolybdc acid into an effective lubricant additive in accordance with the method of the invention, the acid or a salt thereof with a basic organic nitrogen compound, is heated to an elevated temperature above 100° C. and preferably to between 100 and 150° C. with one or more organic reducing compounds of the type described. This heat treatment is carried out until a deep blue color is obtained to indicate completion of the reaction.

In one preferred embodiment, the organic reducing compounds selected for use are those having lubricating properties of their own. The reaction products thus obtained can be added to more of the same lubricants or to other compatible lubricants to adjust the molybdenum concentration to a preselected level. The organic reducing compounds that are particularly useful in this embodiment include, e.g., polyalkylene glycols, their ether or

ester derivatives, dicarboxylic acid esters and higher alcohols.

The molybdenum concentration can vary within wide limits and is ordinarily selected on the basis of the ultimate use of the lubricant being formed. It is generally preferable to adjust the initial content of phosphomolybdc acid or its salts to about 0.1 to 5% by weight based on the total weight of lubricant.

The organic reducing compounds need not be used in precise stoichiometric amounts. They can be used in considerable excess, especially when the reaction products are to be used in mineral oil-based lubricants. In this embodiment, higher alcohols containing ten to eighteen carbon atoms such as dodecanol, hexadecanol and dehydroabietylalcohol are entirely suitable. Eutanol and amines such as oleylamine, dioleylamine, dehydroabietylamine, N-aminopropylmorpholine, di-2-ethylhexylamine and dialkylthioureas, as well as amino alcohols such as oleyloxyethylglyoxalidine and/or mixtures thereof are most effective as reducing agents.

The concentrates thus obtained, which may contain from 10 to 40% of a lubricative molybdenum compound, depending upon the quantity of reducing agent used, increase the lubricating efficiency of liquid lubricants, particularly of mineral oils, in which they are dissolved. They are eminently useful as cutting oils, bearing oils, engine break-in oils, and the like.

If a lubricant is to be subjected to extreme pressures during operation, it may be advisable to introduce sulfur or a sulfur compound before actual use of the lubricant to facilitate reaction *in situ* of molybdenum and sulfur to form molybdenum disulfide. If desired, the sulfur introduced for this purpose may be contained in the reducing compounds used in accordance with the invention for the purpose of reducing the molybdenum from the sexivalent to the tetravalent state and rendering it more soluble in the ultimate lubricant. Sulfur compounds that are suitable for this purpose are, for example, sulfurized unsaturated higher fatty acids and their esters, fatty alcohols, amines, olefinic polymers, organic sulfides and disulfides such as benzylsulfide, dibenzylsulfide, diphenylsulfide as well as xanthates of diols and glycols or dialkylthiourea and phosphorus- and sulfur-containing products such as the derivatives of thiophosphoric acid and dithiophosphoric acid, e.g., zinc dihexylthiophosphate. These and equivalent sulfur-containing compounds are preferably used in proportions of about 0.1 to 5% by weight, based on the combined weight of lubricant.

These and other embodiments of the invention as well as the effectiveness of the additives will become further apparent from the following examples.

#### Example 1

Four percent by weight of phosphomolybdc acid were added to each of the following materials at room temperature:

Ethyl hexanediol  
Abitol  
Eutanol  
n-Octadecanol  
Adipic acid dioctyl diester  
Benzylbutyl phthalate  
Dehydroabietylamine  
"Armeen" 2T  
"Duomeen" C  
"Ucon" 50-HB660  
"Ucon" DLB-67E

Thirty percent by weight of phosphomolybdc acid were added to each of the following materials at room temperature:

Eutanol  
Abitol  
"Flexol" 4GO  
"Flexol" CC-55

The solutions were heated to 125° C., becoming green

upon splitting off water. Further heating to 140° C. caused them to become a deep blue. The solutions were maintained at 140° C. for four days. They were all stable in that no precipitate formed.

#### Example 2

0.05 mol of each of the following amines:

Dehydroabietylamine  
"Armeen" 2T  
"Armeen" SD  
N-aminopropylmorpholine  
Dioleylthiourea

were dissolved in acetone and admixed, while stirring, with 1/140 mols phosphomolybdc acid, likewise dissolved in acetone. A partial precipitation of the resulting phosphomolybdc acid salts took place. Complete recovery of the reaction products was effected by removal of the solvent at 80° C. at reduced pressure.

20 Five grams of each of the salts thus obtained were heated to 150° C. with 10 grams Eutanol. After a total of ten minutes, deep blue solutions were formed which were then subjected to stability tests at 100° C. It was found that after standing for two weeks at this temperature there was no visible precipitation of the salts.

25 Similar tests have been conducted successfully with Abitol, dibutoxytetraglycol, "Ucon" 75-H1400 and a polyethylene glycol having a molecular weight of approximately 500.

#### Example 3

Part A.—A mixture of one p.b.w. (parts by weight) dehydroabietylamine salt of phosphomolybdc acid and 7 p.b.w. Eutanol, prepared as described in Example 2, was added as a concentrate to 92 p.b.w. of a paraffinic raffinate having a viscosity of 17° E. at 50° C. Precipitation of the concentrate began only after the solution had been held at 120° C. for thirty-six hours.

Part B.—In the mixture of Part A, one p.b.w. of the mineral oil was replaced by one p.b.w. of "Armeen" 2T. The mixture was stable for more than ten days at 120° C., showing no precipitation.

Part C.—Five parts of the 30% concentration of phosphomolybdc acid in a mixture of unsaturated ten to eighteen carbon atom alcohols of Example 1 were mixed with 95 parts of a naphthenic spindle oil raffinate having a viscosity of 2° E. at 50° C. Upon standing at 110° C., it began to become cloudy after twenty-four hours.

Part D.—Two parts of a sulfurized dioleylamine containing one mol of sulfur per mol of amine were added to the solution described in Part C. The stability was found to be increased to a showing of no precipitation after standing at least eight days at 110° C.

#### Example 4

55 Several tests were carried out on an Almen Wieland machine (AWM) and a four-ball machine (FBM). The lubricants tested and the results thereof are shown in the table below, in which the term "sulfurized Eutanol" indicates a stoichiometric ratio of one mol Eutanol to 0.5 mol sulfur:

|    |                                                         | AWM,<br>kilograms | FBM,<br>kilograms |
|----|---------------------------------------------------------|-------------------|-------------------|
| 65 | (a) Eutanol.....                                        | 850               | 100/110           |
|    | (b) Eutanol+3% Rosin Amine D.....                       | 700               | 100/110           |
|    | (c) Eutanol+5% Sulfurized Eutanol.....                  | 1,500             | 180/190           |
|    | (d) Eutanol+3% Rosin Amine D+5% Sulfurized Eutanol..... | 1,000             | 130/140           |
|    | (e) a+4% Phosphomolybdc Acid.....                       | 1,500             | 170/180           |
|    | (f) b+4% Phosphomolybdc Acid.....                       | 1,500             | 220/240           |
|    | (g) c+4% Phosphomolybdc Acid.....                       | 1,500             | 260/280           |
| 70 | (h) d+4% Phosphomolybdc Acid.....                       | 1,500             | 320/340           |

<sup>1</sup> Continuous operation.

The data in the table shows that the test results on both machines are improved by the presence of the acidic reaction product of free phosphomolybdc acid as well

as by the mixture that contains excess amine. The increases in lubricating effectiveness after addition of sulfur are practically the same with and without free phosphomolybdc acid whereas with sulfur and a surplus of amine only the molybdenum-containing lubricant shows further improvement.

*Example 5*

*Part A.*—A lubricating mixture was prepared by adding one part of a Rosin Amine D-phosphomolybdate in 3 p.b.w. Abitol and 3 p.b.w. Eutanol to 93 p.b.w. of a naphthenic raffinate having a viscosity of 17° E. at 50° C. This mixture was found to be stable for three days at 110° C. and then slowly became cloudy. It was slightly corrosive to ferrous and non-ferrous metals. Upon testing on the Almen Wieland machine under continuous operation at a load of 1500 kgs., a constant friction coefficient of 0.133 was measured. The four-ball machine test indicated 170/180 kgs.

*Part B.*—One-half part of the naphthenic raffinate of the mixture of Part A was replaced by an equal amount of "Armeen" 2T. The stability at 110° C. was thereby increased to at least ten days and the mixture was no longer corrosive to ferrous and non-ferrous metals. In continuous operation on the Almen Wieland machine with a 1500 kg. load, a constant coefficient of friction of 0.125 was made. The four-ball value was 180/190 kg.

*Part C.*—One-half of the naphthenic raffinate of the mixture in Part A was replaced by an equal amount of sulfurized "Armeen" 2T, the sulfur content being one mol per mol of "Armeen." The heat stability was the same as in Part B but the mixture was found to be somewhat corrosive to non-ferrous metals. At constant operation on an Almen Wieland machine at 1500 kgs. load, a coefficient of friction of 0.13 was measured. The four-ball value was increased to 240/260 kg.

*Part D.*—A lubricating mixture was prepared by adding a concentrate containing 0.7 p.b.w. phosphomolybdc acid, 1.3 p.b.w. dioleylthiourea and 6 p.b.w. Abitol to 92 p.b.w. naphthenic raffinate having a viscosity of 17° E. at 50° C. The mixture remained stable for eight days at 110° C. and showed slight corrosive action with non-ferrous metals. Under continuous operation on an Almen Wieland machine at a load of 1500 kgs., a coefficient of friction of 0.12 was measured. The four-ball value was 230/240 kg.

*Example 6*

Two oils were prepared which differed from one another only in the amount of sulfur in the form of zinc dihexylthiophosphate. They had the following formulations:

|                                             | Oil A,<br>Parts | Oil B,<br>Parts |
|---------------------------------------------|-----------------|-----------------|
| Rosin Amine D-phosphomolybdate              | 1               | 1               |
| "Armeen" 2HT                                | 1               | 1               |
| Eutanol                                     | 7               | 7               |
| Tech. zinc dihexylthiophosphate concentrate | 2               |                 |
| Naphthenic raffinate                        | 91              | 89              |

Both oils were found to be stable for fourteen days at 110° C. and neither of them showed any corrosion on ferrous or non-ferrous surfaces. The Almen Wieland value was determined with regular bearings and the coefficient of friction of both oils under continuous operation at loads of 1500 kgs. was found to be 0.12. Another test run with hardened bearings showed no materially different behavior, both oils showing a load capacity of up to 2500 kgs. with equal friction curves. The four-ball values of oils A and B, however, were 160/170 and 240/260 kgs., respectively, showing an increase due to the presence of sulfur.

The two oils were further subjected to the Niemann test for hypoid gear oils. Oil A reached eight load levels with a specific wear of between 0.1 and 0.2 mgs. per horse-

power hour whereas oil B endured twelve load levels, which is the maximum possible with this test. The specific wear was between 0.05 and 0.1 mgs. per horsepower hour.

We claim:

- 5 1. A method which comprises heating (A) a member of the group consisting of phosphomolybdc acid and a salt thereof with an organic nitrogen base of the group consisting of oleyloxyethylglyoxalidine, N-aminopropylmorpholine and primary and secondary hydrocarbon and hydrocarbon acyl amines with (B) an organic reducing compound of the group consisting of high molecular weight alkylene glycols, abietyl alcohols, alkyl alcohols, carboxylic acid esters and polyalkylene glycols having at least eight carbon atoms to a temperature between about 100 and 150° C. until the reactants assume a deep blue color, the amount of reactant B being sufficient to reduce at least a part of the molybdenum to tetravalent form.
- 10 2. The method defined in claim 1 wherein the organic reducing compound has lubricating properties.
- 15 3. The method defined in claim 1 in which the organic reducing compound is used in excess of the amount stoichiometrically required to reduce the valence of the molybdenum therein from six to four.
- 20 4. The method defined in claim 1 wherein the reaction is carried out in the presence of an excess amount of a free nitrogen base of the group consisting of oleyloxyethylglyoxalidine, N-aminopropylmorpholine and primary and secondary hydrocarbon and hydrocarbon acyl amines of 8 to 18 carbon atoms, said amount being in excess of the amount required to reduce the valence of the molybdenum therein from six to four.
- 25 5. A method which comprises neutralizing phosphomolybdc acid by reaction with an organic nitrogen base of the group consisting of oleyloxyethylglyoxalidine, N-aminopropylmorpholine and primary and secondary hydrocarbon and hydrocarbon acyl amines of 8 to 18 carbon atoms and reducing the resulting salt with an organic reducing compound of the group consisting of high molecular weight alkylene glycols, abietyl alcohols, alkyl alcohols, carboxylic acid esters and polyalkylene glycols having at least eight carbon atoms at a temperature between about 100 and 150° C. until the reactants assume a deep blue color.
- 30 6. A method which comprises heating phosphomolybdc acid with an amount of an organic nitrogen base of the group consisting of oleyloxyethylglyoxalidine, N-aminopropylmorpholine and primary and secondary hydrocarbon and hydrocarbon acyl amines of 8 to 18 carbon atoms in stoichiometric excess of the amount required to form a neutral salt thereof for neutralizing and reducing said acid to a non-corrosive, lubricant-soluble state.
- 35 7. A method which comprises heating phosphomolybdc acid with a non-basic organic reducing compound of the group consisting of high molecular weight alkylene glycols, abietyl alcohols, alkyl alcohols, carboxylic acid esters and polyalkylene glycols having at least eight carbon atoms to a temperature between about 100 and 150° C. until the reactants assume a deep blue color and become lubricant-soluble, and neutralizing said reduced product by reaction with an organic nitrogen base of the group consisting of oleyloxyethylglyoxalidine, N-aminopropylmorpholine and primary and secondary hydrocarbon and hydrocarbon acyl amines 8 to 18 carbon atoms.
- 40 8. The product prepared by the method defined in claim 1.
- 45 9. The product defined in claim 8 wherein the organic nitrogen base contains sulfur.
- 50 10. A lubricating oil selected from the group consisting of mineral and polyalkylene glycol lubricating oils containing about 0.1 to 5% by weight of an additive prepared by the method defined in claim 1.
- 55 11. The product prepared by the method defined in claim 1 wherein the organic reducing compound is ethyl hexanediol.
- 60 12. The product prepared by the method defined in

claim 1 wherein the organic reducing compound is a di-octyl diester of adipic acid.

13. The product prepared by the method defined in claim 1 wherein the organic reducing compound is a di-octyle diester of suberic acid.

14. The product prepared by the method defined in claim 1 wherein the organic reducing compound is benzyl-butyl phthalate.

15. A product prepared by heating a salt of phosphomolybdic acid and N-aminopropylmorpholine with di-butoxytetraglycol to a temperature between about 100 and 150° C. until the reactants assume a deep blue color.

16. A product prepared by heating a salt of phosphomolybdic acid and N-aminopropylmorpholine with a poly-ethylene glycol having a molecular weight of about 500 to a temperature between about 100 and 150° C. until the reactants assume a deep blue color.

## References Cited in the file of this patent

## UNITED STATES PATENTS

|           |                     |                |
|-----------|---------------------|----------------|
| 2,788,258 | Arnold et al. ----- | Apr. 9, 1957   |
| 2,852,469 | Hugel -----         | Sept. 16, 1958 |
| 2,900,235 | Arnold et al. ----- | Aug. 18, 1959  |

## OTHER REFERENCES

Lieboff: "Reduction of Phosphomolybdic Acid by Monomethyl-p-Amino Phenol," Chem. Abstracts 25: 26607, 1931.

Tschopp et al.: "The Reduction of Phosphomolybdic Acid to Molybdenum Blue," Chem. Abstracts 26: 51128, 1932.

Bannann et al.: "A New Reaction at the Naphthionic Acid Molecule," Chem. Abstracts 47: 9949i, 1953.